

## UNITED STATES PATENT OFFICE

2,514,650

## PHOTOGRAPHIC DEVELOPING WITH ADDITION PRODUCTS TO IMPROVE IMAGE QUALITY

Edward Bowes Knott and John Morgan, Wealdstone, England, assignors to Eastman Kodak Company, Rochester, N. Y., a corporation of New Jersey

No Drawing. Application March 27, 1947, Serial No. 737,710. In Great Britain April 5, 1946

14 Claims. (Cl. 95-7)

**1** This invention relates to photographic materials and more particularly to a method of improving the quality of the developed images given by photographic silver salt emulsions.

The development of exposed silver halide photographic emulsions leads to the formation of a silver image which may vary considerably in colour depending on the type of silver halide, the size of the silver halide grain and on the type of developer used. Generally, the finer the developed grain the greater is the tendency for the image to appear brown or green-brown in colour but in many cases it is desirable that the image should be a neutral grey or black or blue-black.

Another undesirable feature which is often experienced is the liability of the developed image to the effect known as "plumming" or "bronzing" which occurs during the hot-glazing of prints and produces an adverse effect on image colour and density.

A large number of emulsion and developer addition agents have been described which prevent the formation of coloured images or act as anti-plumming agents but the large majority of such compounds suffer from the disadvantage that they are effective only in silver chloride emulsions. Certain agents which are also effective in silver bromide emulsions have the disadvantage that they are active only after the emulsion containing the agent has been incubated or held a considerable time after coating. Among these agents are some which, at the same time, are also hardening agents and it is not always possible to obtain the correct hardness with effective toning.

It is accordingly an object of our invention to provide a novel method of producing developed photographic images of improved quality. Another object is to provide substances which, besides acting as antifogging agents for silver halide emulsions in general, also produce very desirable blue-black tones on development. Yet another object is to provide a method of preventing or reducing plumping or bronzing of prints during the hot-glazing process. Another object is to provide novel photographic materials and developers for producing developed images of improved quality. These and other objects will be apparent from the following specification.

We have now found a method of producing developed photographic images of improved quality from a photographic material having a sensitive silver halide emulsion layer which comprises processing the said material in the presence of a

**2** compound selected from the group represented by the following general formula:



wherein **X** represents a divalent organic group and **Y** represents a member selected from the group consisting of ureido groups, substituted ureido groups, and nitrogen-containing heterocyclic groups having from five to six atoms in the heterocyclic ring. For example, **X** may represent a carbon chain such as alkylene, e. g. methylene, ethylene, trimethylene, or the like, or substituted alkylene, or methine, or polymethine, or a hetero-carbon chain, or a group comprising a carbocyclic component, e. g. ortho-, meta-, or para-xylene, or a heterocyclic component; **Y** may represent a ureido-group represented by the formula:



wherein **R**, **R'** and **R''** each represent a group selected from the class containing hydrogen, alkyl, aryl and aralkyl groups, or a heterocyclic group having the formula:



**30** wherein **Z** represents the non-metallic atoms necessary to complete a heterocyclic nucleus containing from five to six atoms in the heterocyclic ring, e. g. imidazole, dihydroimidazole, benzimidazole, pyrimidine, thiodiazine, thiodiazole, or the like.

Substances in which **Y** represents ureido or substituted ureido are preferably employed as their salts or quaternary salts which are usually more stable than the bases and are water soluble.

**40** These salts are usually readily obtained by heating substances of the type:



**45** with dihalogen derivatives **X(Hal)<sub>2</sub>** according to the equation:



In the above equation the symbols X, R, R', R'' have the same meaning as before.

These substances of the invention are added preferably to the emulsion layer or layers but they are also effective, when of the requisite solubility, if added to the developing solution or to other layers carried on the sensitive emulsion support such as the backing layer or supercoat. Alternatively the sensitive layer may be bathed in a solution of the agent after exposure but prior to development. The substance is added to the emulsion layer preferably in amounts corresponding to 1-10 g. for every 127 g. of silver or to a developer at the rate of 0.2-2.0 g./litre. Higher concentrations of the agent may be used without increasing the effect.

Many of these agents have the advantage of giving neutral images in freshly coated material and it is unnecessary to hold the sensitive layer for long periods, or to incubate them to produce the effect. The optimal concentration for such immediate effects is 2-5 g. agent for every 127 g. silver in the emulsion. At lower concentrations these same agents give their best effect on incubating the sensitive layer containing them.

The compounds according to the invention are also valuable for preventing or reducing the overall silver deposit termed "fog" which is frequently obtained on developing silver halide emulsion. To produce this antifoggant effect concentrations as low as 0.10 gram per 127 grams of silver may be used, but at these low concentrations there is very little effect on the colour of the image.

The compounds are very effective as anti-plumming agents when used in any of the ways previously described or by bathing the developed image in a solution of the compound after fixation. A suitable bath is, for example, an aqueous solution containing from 0.2 to 2.0 grams/litre of the anti-plumming agent.

Although in the specification we have described our invention mainly with reference to the use of our new agents in developing solutions and anti-plumming baths it should be understood that our invention is by no means limited to such baths. Where the term "processing" is used in this specification we include any treatment given to the photographic material after exposure and up to the production of the final washed image and, in the case of prints especially, including the final hot-glazing treatment. Thus, although the agent is preferably added in the developing solutions (when not already present in the photographic material) it may be added in the fixing bath or prior to washing since sufficient of the compound will be adsorbed to the silver grains to give the desired anti-plumming effect during hot-glazing of the print.

Our invention is illustrated by the following examples of compounds which may be used, together with their methods of preparation and use:

#### EXAMPLES OF PREPARATION

##### Example I.—S:S'-methylene-bis-thiuronium iodide



See Dixon and Taylor, J. Chem. Soc. 1916, 109, 1255.

##### Example II.—S:S'-ethylene-bis-thiuronium bromide



See Andreasch, Monatshefte der Chemie, 1883, 4, 142; Schatzmann, Annalen der Chemie, 1891, 261, 4.

##### Example III.—S:S'-trimethylene-bis-thiuronium bromide



Thiourea (7.6 g.), 1:3-dibromopropane (5.6 c. c.), and ethyl alcohol (50 c. c.), are refluxed for 3 hours. On allowing the liquor to cool the salt crystallized. It formed needles, M. P. 198°, after washing with alcohol.

##### Example IV.—2:2'-methyleneethio-bis-dihydro-iminazole dihydriodide



Ethylenethiourea (2-thiotetrahydroiminazole) (Schacht, Arch. der Pharm., 1897, 235, 442; Klut, ibid., 1902, 240, 675) (10.2 g.), methylene iodide (13.4 g.) and ethyl alcohol (75 c. c.) were refluxed for 2 hours. Crystallization occurred during the refluxing. The crystals were collected after cooling and washed with alcohol. They formed colourless needles, M. P. 240°.

##### Example V.—2:2'-ethylenethio-bis-dihydro-iminazole dihydriobromide



Ethylenethiourea (10.2 g.), ethylenedibromide (9.4 g.) and ethyl alcohol (100 c. c.) were refluxed for 2 hours and the precipitated crystals filtered off from the hot liquor. It formed colourless needles of no definite melting point. The base released by alkali had M. P. 203° from methyl alcohol (Schacht, loc. cit., p. 455).

##### Example VI.—2:2'-trimethyleneethio-bis-dihydro-iminazole dihydriobromide



Ethylenethiourea (10.2 g.) was dissolved in boiling ethyl alcohol (100 c. c.) and 1:3-dibromopropane (5.6 c. c.) added and the whole refluxed for 3 hours. The salt was collected after allowing the mixture to cool, and after washing with alcohol had M. P. 224°.

##### Example VII.—2:2'-ethylenethio-bis-(4-methyl-dihydroiminazole) dihydriobromide



2-thio-4-methyltetrahydroiminazole (Johnson and Edens), J. Amer. Chem. Soc. 1942, 64, 27027) (3.5 g.), ethylene dibromide (1.3 c. c.) and ethyl alcohol (25 c. c.) were refluxed for 2 hours. On chilling the required dihydriobromide separated. It was collected, boiled up with ethyl alcohol and

filtered from the hot liquor. It formed a white crystalline powder, M. P. 236°.

*Example VIII.—2:2'-trimethylenethio-bis-(4-methyliminazole) dihydrobromide*



2-thio-4-methyltetrahydrominazole (3.5 g.), 1:3-dibromopropane (1.55 c. c.) and ethyl alcohol (25 c. c.) were refluxed for 2 hours. To the cold solution ether was added to precipitate a thick oil which slowly crystallized. The ether-alcohol was decanted, the crystals washed with cold alcohol and dissolved in boiling ethyl alcohol. The slow addition of ether gave colourless needles of the salt, M. P. 177°.

*Example IX.—Disodium-2:2'-ethylenethio-bis-(4-amino-6-hydroxypyrimidine)*



The di-sodium salt of 2-thiol-4-amino-6-hydroxypyrimidine (18.7 g.) was dissolved in water (20 c. c.) and ethylene bromide (5 c. c.) and spirit (50 c. c.) added and the whole refluxed for 1 hour. The solution was concentrated and the pale yellow solid of indefinite melting point collected, washed with alcohol and ether and dried.

*Example X.—S:S'-ethylene-bis-N-ethyl-thiuronium bromide*



Ethylthiourea (5.2 g.), ethylene dibromide (2.5 c. c.) and ethyl alcohol (20 c. c.) were refluxed for 1 hour. Dry ether was slowly added with shaking to give a mass of white crystals. They were collected, washed with alcohol-ether (1:2) then with ether. M. P. 92°. They are very hydroscopic.

*Example XI.—S:S'-ethylene-bis-N:N'-diethyl-thiuronium bromide*



(Noah, Ber., 1890, 23, 2198). S-diethylthiourea (6.6 g.), ethylene dibromide (2.5 c. c.) and ethyl alcohol (20 c. c.) were refluxed for 1 hour. Dry ether was slowly added with shaking to give a mass of crystals. They were collected, washed with alcohol-ether (1:2) then with ether. M. P. 186°.

*Example XII.—S:S'-trimethylene-bis-N:N'-triethylthiuronium bromide*



See Noah, Ber., 1890, 23, 2200.

*Example XIII.—S:S'-ethylene-bis-N:N'-triethylthiuronium bromide*



Triethylthiourea (8.0 g.), ethylene dibromide (2.5 c. c.) and ethyl alcohol (20 c. c.) were refluxed for 2 hours, chilled and the salt precipitated as an oil with dry ether. The ether was decanted and the process repeated shaking vigorously after each addition. The thick oil so obtained crystallized slowly on standing under ether. It was collected, drained well, dissolved in ethyl alcohol and reprecipitated with ether.

10 It formed white needles, M. P. 130-132°.

*Example XIV.—S:S'-o-xylylenyl-bis-thiuronium bromide*



o-Xylylenedibromide (5.3 g.), thiourea (3.0 g.), and ethyl alcohol (25 c. c.) were refluxed for 90 minutes. Ether was added to precipitate an oil which crystallized. It formed soft needles, M. P. 225-226° after recrystallization from a little water and acetone.

*Example XV.—S:S'-ethylenethio-bis-(1-methyl-dihydroiminazole) di-p-toluenesulphonate*



On warming 2:2'-ethylenethio-bis-dihydroiminazole (1 mol.) with methyl p-toluenesulphonate (2 mol.) on the steam bath a vigorous reaction ensued and a thick oil remained. This is completely water soluble and is believed to have the above constitution.

40 *Example XVI.—S:S'-ethylene-bis-N-phenyl-N-methylthiuronium bromide*



N-phenyl-N-methylthiourea (3.3 g.), ethylene dibromide (1 c. c.) and ethyl alcohol (10 c. c.) were refluxed for 2 hours. The addition of ether precipitated a gum which was washed with ether and recrystallized from spirit-ether forming needles M. P. 214°.

55 *Example XVII.—4:4'-ethylenethio-bis-(4:6-dithio-1:3:5-thio diazine)*



60 2:4:6-trithio-1:3:5-thiodiazine (0.97 g.) and ethylene dibromide (0.21 c. c.) were dissolved in ethyl alcohol (10 c. c.) and refluxed for 1 hour during which fine white crystals were formed.

65 They were filtered off, and recrystallized from aqueous alcohol, as fine white needles M. P. 231°.

*Example XVIII.—2:2'-ethylenethio-bis-(5-thiol-1:3:4-thiodiazole)*



70 2:5-dithiol-1:3:4-thiodiazole (3.0 g.) was dissolved in ethyl alcohol (15 c. c.) and ethylene di-

75 solved in ethyl alcohol (15 c. c.) and ethylene di-

bromide (0.86 c. c.) added. After refluxing for 5 hours, during which fine white crystals appeared, the mixture was cooled and filtered. The solid was recrystallized from aqueous alcohol as white prisms M. P. 254°.

#### EXAMPLES OF USE

*Example A.*—5 g. of the compound of Example I added to 5 litres of a fine grained positive type emulsion (containing the equivalent of 200 g. silver nitrate) changes the normal olive brown tone of the blacks to blue black when developed in a normal metol-hydroquinone developer.

*Example B.*—2 g. of the compound of Example II added to 5 litres of this emulsion gave almost neutral blacks while 5 g. in the same quantity gave pronounced blue blacks. Incubation for 3 days at 50° C. of the coated emulsion caused a further change of tone towards the blue shades.

*Example C.*—5 g. of the compound of Example III added to 8 litres of a chloride emulsion (containing the equivalent of 200 g. silver nitrate) changed the brown tone of the blacks to blue-black.

*Example D.*—The addition of 1 g. of the compound of Example II per litre of normal metol-hydroquinone developer when developing the fine grained positive emulsion, as used in Examples A and B, gave blacks only faintly brown, compared with the pronounced olive brown tones normally obtained.

*Example E.*—5 g. of the compound of Example III added to 5 litres of the fine grained positive emulsion gave the blue tone to the black when developed in a normal metol-hydroquinone developer.

*Example F.*—5 g. of the compound of Example IV added to 5 litres of the fine grained positive emulsion produced very strong blue-black effect.

*Example G.*—3 g. of the compound of Example V added to 5 litres of the emulsion used for the previous example reduced the brown tone of the blacks, while 5 g./5 litres gave nearly neutral blacks. Incubation of the coated plates for 3 days at 50° C. resulted in a further effect giving blue-black on development.

*Example H.*—5 g. of the compound of Example VI added to 5 litres of the same emulsion reduced the brown tones giving nearly neutral blacks with normal metol-hydroquinone development.

*Example J.*—5 g. of the compound of Example VII added to 5 litres of the same emulsion gave a similar effect to Example H initially; but incubation for 3 days at 50° C. caused increase in effect giving definite blue blacks.

*Example K.*—5 g. of the compound of Example IX added to 5 litres of the emulsion used above gave good blue black tones on normal development.

*Example L.*—5 g. of the compound of Example X added to 5 litres of the emulsion used above gave almost neutral blacks on development; after incubation for 3 days at 50° C. the blacks obtained were slightly bluish.

*Example M.*—5 g. of the compound of Example XI added to 5 litres of the emulsion gave a similar result to Example L initially, but after incubation very strong blue black tones were obtained on development.

*Example N.*—5 g. of the compound of Example XIII added to 5 litres of the emulsion gave almost identical results with those in Example L.

*Example O.*—5 g. of the compound of Example XIV added to 5 litres of the emulsion gave neutral blacks on development.

*Example P.*—5 g. of the compound of Example XV added to 5 litres of the same emulsion gave strong blue-black tones.

*Example Q.*—(a) A silver chloro-bromide emulsion coated on paper was exposed to a step wedge, developed, and fixed.

(b) The same paper was treated as above but with the addition of 1 g. of the compound of Example II to 1 litre of developer.

(c) The same paper was treated as in (a) but after fixation the paper was bathed in a solution of 5 g. of the compound of Example I in 100 c. c. water for 5 minutes.

On hot-glazing, the papers treated according to (b) or (c) gave very deep blacks whilst the untreated paper (a) showed a big loss of density.

*Example R.*—On substituting the compound of Example XIII for that of Example II in Example Q (b) a similar effect was obtained.

*Example S.*—On substituting the compound of Example V for that of Example II in Example Q (c) a similar effect was obtained.

*Example T.*—A high speed panchromatic emulsion was coated: (a) as such with the usual hardener; (b) as (a) but with the addition of 0.25 g. of the compound of Example II per 5 litres of emulsion containing the equivalent of 200 g. silver nitrate. On forced development or after incubation the coating (a) showed a much higher fog than did (b).

Other agents such as those of Examples II, V, VI, VII, X, XI, XII, etc., added to the emulsion at the same rate also showed pronounced antifogging and stabilizing properties.

*Example U.*—A silver chloride emulsion was divided and one part coated on paper. The other part was melted and to an amount of the emulsion containing the equivalent of 200 g. silver nitrate was added 8 g. of the compound of Example II and the emulsion coated.

After exposure and processing, strips of the two coatings were hot glazed. Those strips containing the agent showed a much blacker and high maximum density than the strips coated with the untreated emulsion.

*Example V.*—Substitution of the same quantity of the compound of Example XVII for the compound of Example II in the experiments of Example U gave similar results.

*Example W.*—Substitution of the same quantity of the compound of Example XVIII for the compound of Example II in the experiments of Example V gave similar results and the increase in maximum density was particularly good in this case.

Having thus described our invention what we claim is:

1. Method of producing developed photographic images of improved quality from a photographic material having a sensitive silver halide emulsion layer comprising developing the said material in the presence of a compound selected from the group represented by the following general formulae:



and



where X represents a divalent organic group selected from the class consisting of alkylene and



11

graphic images of improved quality having a sensitive silver halide emulsion layer comprising developing said material in the presence of a compound having the formula:



12. A photographic material comprising a sensitive silver halide emulsion layer containing 10 the quaternary salt of a compound having the following formula:



where  $\text{X}$  represents an alkylene group.

13. A photographic material comprising a sensitive silver halide emulsion layer containing the quaternary salt of a compound having the 20 following formula:



where  $\text{X}$  represents an alkylene group and  $\text{R}$  represents an alkyl group.

12

14. A photographic material comprising a sensitive silver halide emulsion layer containing a compound having the formula:



where  $\text{X}$  represents an alkylene group.

EDWARD BOWES KNOTT,  
JOHN MORGAN.

#### REFERENCES CITED

The following references are of record in the file of this patent:

#### UNITED STATES PATENTS

| Number    | Name          | Date          |
|-----------|---------------|---------------|
| 2,124,159 | Weyde         | July 19, 1938 |
| 2,453,087 | Dersch et al. | Nov. 2, 1948  |
| 2,465,149 | Dersch et al. | Mar. 22, 1949 |

#### OTHER REFERENCES

Kraft: "Zeit für Wiss. Phot." Bd. 31, Heft 12, May 1932, pages 329 to 364, pages 353 and 355 cited.